

# United States Patent

[19]

[11] 3,753,026

Goorissen

[45] Aug. 14, 1973

## [54] QUARTZ LAMP SEAL

[75] Inventor: Jan Goorissen, Emmasingel,  
Eindhoven, Netherlands[73] Assignee: U.S. Philips Corporation, New York,  
N.Y.

[22] Filed: Dec. 7, 1970

[21] Appl. No.: 95,436

## [30] Foreign Application Priority Data

Dec. 13, 1969 Netherlands ..... 6918746

[52] U.S. Cl. ..... 313/318, 313/332

[51] Int. Cl. ..... H01J 5/38, H01J 5/46, H01J 5/52

[58] Field of Search ..... 313/315, 317, 318,  
313/332; 174/50.64

|           |         |                       |             |
|-----------|---------|-----------------------|-------------|
| 3,617,797 | 11/1971 | Meijer et al. ....    | 313/318     |
| 2,992,959 | 7/1961  | Schrewelius ....      | 338/330     |
| 3,681,737 | 8/1972  | Magnusson et al. .... | 338/330     |
| 3,105,867 | 10/1963 | Meijer.....           | 174/50.64   |
| 3,669,693 | 6/1972  | Dalton et al. ....    | 117/201     |
| 3,549,933 | 12/1970 | Smalley.....          | 313/318 X   |
| 2,113,984 | 4/1938  | Harris et al. ....    | 174/50.64 X |
| 3,515,420 | 6/1970  | Thomasson et al. .... | 174/50.64 X |
| 3,211,826 | 10/1965 | Holcomb et al. ....   | 313/318 UX  |

Primary Examiner—Rudolph V. Rolinec

Assistant Examiner—Marvin Nussbaum

Attorney—Frank R. Trifari

## [57] ABSTRACT

An electric lamp including an envelope of quartz glass in which at least part of the metal components sealed in the pinch is coated with  $\text{SiO}_2$ .

## 4 Claims, 5 Drawing Figures

## [56] References Cited

## UNITED STATES PATENTS

3,420,944 1/1969 Holcomb ..... 174/50.64



PATENTED AUG 14 1973

3,753,026



Fig. 1



Fig. 2



Fig. 3



Fig. 4



Fig. 5

INVENTOR.  
JAN GOORISSEN

BY  
Leand R. Sijpwi  
AGENT

## QUARTZ LAMP SEAL

The invention relates to an electric lamp including an envelope of quartz glass or a similar high melting-point material which is transparent to light and has a low thermal coefficient of expansion, which lamp includes at least one pinch in which at least one strip consisting of a metal foil is sealed in, at least one current conductor of metal wire being secured by means of welding to both ends of said strip, while one conductor serves as an electric contact for the lamp. The foil consists of a metal having a melting point of more than 1,500°C so that during sealing in the foil cannot melt. For this use a metal is chosen having a low thermal coefficient of expansion. Usually the foil consists of tungsten, molybdenum or a suitable alloy of tungsten and molybdenum.

In lamps of this kind a strip in the form of foil of such a metal is used in the pinch because it has been found that in spite of the difference in coefficient of expansion between quartz glass on the one hand and the metal on the other hand a gastight closure can be obtained therewith.

The construction of the pinch in question is frequently used in high-power lamps such as infrared radiators and halogen lamps in which not only the envelope but also the pinches may assume a high temperature when the lamps are operating.

During the manufacture of the pinch a capillary space is substantially always formed around that part of the current conductor partially extending beyond the lamp which is present within the pinch.

In high-power lamps the pinch often cracks during use. This is generally ascribed to an oxidation of the current conductor partially extending beyond the lamp and of the metal foil strip. This oxidation is caused by oxygen and water vapour from the air which may reach the foil through the capillary along this conductor.

Various steps have been proposed to protect the portion of the conductor extending beyond the lamp and being present within the pinch and the metal foil strip against oxidation. The object of the proposed steps is either to enhance the adhesion between quartz and the metal parts or to provide the metal parts with an oxidation-protective layer. The materials used for this purpose are metals or metal oxides which cannot be oxidized at the temperature of the pinch. In practice these steps were not found to be successful because it was still difficult to obtain a permanently gastight closure when using these materials.

An object of the present invention is to provide an electric lamp in which cracking of the pinch as a result of oxidation of metal parts in the pinch does not occur or substantially does not occur.

It was found that this may be achieved with a lamp which is characterized in that at least the part located within the pinch of the current conductor partially protruding from the lamp, the area where this conductor is secured to the metal foil strip and at least the part of this strip adjacent to the area of securement are coated with a thin film of  $\text{SiO}_2$ .

For achieving the desired effect an  $\text{SiO}_2$  film having a thickness of from 0.5  $\mu\text{m}$  to 2  $\mu\text{m}$  is found to be amply sufficient.

The present invention is particularly interesting for those lamps in which the temperature of the pinch during use assumes a value of more than approximately 300°C and consists of molybdenum foil.

In order that the invention may be readily carried into effect some embodiments thereof will now be described in detail by way of example with reference to the accompanying diagrammatic drawing in which

5 FIG. 1 shows a molybdenum strip including current conductors, which strip is partially coated with  $\text{SiO}_2$ .

FIG. 2 is a cross-section taken on the line II-II of FIG. 1.

10 FIG. 3 shows a molybdenum strip including current conductors, which strip is completely coated with  $\text{SiO}_2$ .

FIG. 4 is a cross-section taken on the line IV-IV of FIG. 3 according to the invention.

15 FIG. 5 shows a cross-section of part of a halogen lamp.

FIG. 1 shows in a plan view a molybdenum strip 1 to which a molybdenum current conductor 2 and the end of the filament 3 are secured by means of welding. Part of the current conductor 2 and part of the molybdenum strip 1 are coated with a thin film 4 of  $\text{SiO}_2$  which is obtained by sputtering.

FIG. 2 shows in a side elevational view a cross-section taken on the line II-II of FIG. 1. The thickness of the film 4 is approximately 1  $\mu\text{m}$ . This construction is used if after providing the  $\text{SiO}_2$  film something else is to be secured to the molybdenum strip by means of welding.

FIG. 3 shows in a plan view a molybdenum strip 5 to which two current conductors 6 and 7 are secured by means of welding. Part of the conductors 6 and 7 and the strip 5 are coated with a thin film of  $\text{SiO}_2$  (8) which is provided by means of sputtering. After the strip 5 and the conductors 6 and 7 welded thereto are coated with  $\text{SiO}_2$ , the filament 9 is secured to the conductor 8.

FIG. 4 shows a cross-section taken on the line IV-IV of FIG. 3.

The thickness of the  $\text{SiO}_2$  film is in this case likewise approximately 1  $\mu\text{m}$ . The  $\text{SiO}_2$  films were obtained by means of sputtering in an argon atmosphere at a pressure of approximately  $2 \times 10^{-3}$  Torr. The rate of application was approximately 250 A per minute. A voltage of several kV was applied with the aid of a high-frequency generator (1 kw, frequency 20 MC) between the cathode and the substrate to be coated. The parts of the molybdenum strip and the conductors secured thereto which were not to be coated with  $\text{SiO}_2$  were covered with a mask.

FIG. 5 shows in a cross-section a part of a halogen lamp (1,000 W, 125 Volts) whose pinch temperature 50 during operation of the lamp may increase to approximately 400°C in certain types of reflectors. The thickness of the molybdenum foil 10 is approximately 35  $\mu\text{m}$ . A thin film 11 of  $\text{SiO}_2$  (approximately 1  $\mu\text{m}$  thick) is provided on the molybdenum foil, which film also extends beyond the pinch over approximately 5 mm on the molybdenum conductor 12. The lamp includes a spiral 13 in an atmosphere consisting of argon and a small quantity of iodine (total pressure 2.5 atmospheres). The lifetime of this lamp is approximately 60 2,000 hours.

Number of lumens/Watt: 22. If there is no  $\text{SiO}_2$  film oxidation in the pinch 14 occurs already after a short period in many cases followed by cracking of the pinch. When using the film of  $\text{SiO}_2$  no oxidation in the pinch of the molybdenum parts can be found, not even at the end of the lifetime of the lamp.

What is claimed is:

1. In an electric lamp of the type having an envelope of a high melting-point material such as quartz glass, which is transparent to light and has a low thermal coefficient of expansion, which lamp includes at least one pinch in which at least one strip consisting of a metal foil is sealed in, at least one current conductor of metal wire being secured by means of welding to each end of said strip, one conductor serving as an electric contact for the lamp wherein the improvement comprises that a thin film of  $\text{SiO}_2$  forms a coating over the portion of the contact serving current conductor which is located

within the pinch, the area where this conductor is secured to the metal foil strip, and the part of this strip adjacent the area of securement.

2. An electric lamp as claimed in claim 1, wherein the thickness of the  $\text{SiO}_2$  film is between 0.5 and 2  $\mu\text{m}$ .

3. An electric lamp as claimed in claim 1, wherein said metal foil is molybdenum.

4. The lamp as claimed in claim 1 wherein said thin film of  $\text{SiO}_2$  forms a coating over the entire metal foil strip and the ends of the conductors.

\* \* \* \* \*

15

20

25

30

35

40

45

50

55

60

65